



EXAMPLE 5  
*Flotation of a copper ore*

In order to show the utility of the dithiocarbamates of the present invention as flotation promoters, the compounds of Examples 1, 2 and 3 were employed in the recovery of copper from an ore from the western United States, using the following procedure. The ore sample was ground for 5 minutes at 60% solids with 0.03 lb./ton of promoter (pH 7.8). It was then conditioned for one minute with 0.09 lb./ton of cresylic acid and 0.025 lb./ton of fuel oil. The pulp was floated for 8 minutes and the tailing analyzed for residual copper, with the following results.

TABLE I

| No.    | Compound       | Percent Cu in Tailing |
|--------|----------------|-----------------------|
| 1..... | Example 1..... | 0.19                  |
| 2..... | Example 2..... | 0.34                  |
| 3..... | Example 3..... | 0.19                  |

I claim:

1. A compound of the following formula:



wherein R and R' are individually selected from the group consisting of alkyl of up to eighteen carbons containing up to about three substituents selected from the group consisting of chloro, bromo, fluoro, nitro, cyano, lower alkoxy and amino; phenyl, naphthyl and diphenyl having up to about five substituents selected from the group consisting of chloro, bromo, fluoro, lower alkyl, cyano, amino, nitro and lower alkoxy; and benzyl and naphthylmethyl having up to about three substituents selected from the group consisting of chloro, fluoro, bromo, lower alkyl, cyano, lower alkoxy, amino and nitro.

- 5 2.  $\beta$ -Cyanovinyl diethyldithiocarbamate.  
10 3.  $\beta$ -Cyanovinyl di-n-butylidithiocarbamate.  
15 4.  $\beta$ -Cyanovinyl-N-benzyl-N-methyldithiocarbamate.

## References Cited by the Examiner

## UNITED STATES PATENTS

|    |           |       |               |       |            |
|----|-----------|-------|---------------|-------|------------|
| 20 | 2,231,265 | 2/41  | Gaudin        | ----- | 209—167    |
|    | 2,512,669 | 6/50  | Morrow        | ----- | 209—167    |
|    | 2,854,467 | 9/58  | Harman et al. | ----- | 260—455    |
|    | 2,901,498 | 8/59  | Tilles et al. | ----- | 260—455    |
|    | 2,914,547 | 11/59 | Gaertner      | ----- | 260—455 XR |

25 CHARLES B. PARKER, Primary Examiner.